

# United States Patent

Ohlbaum et al.

[15] 3,653,940

[45] Apr. 4, 1972

[54] **TITANIUM AND TITANIUM ALLOY  
WITH LUBRICANT COATED SURFACE**

[72] Inventors: Robert A. Ohlbaum, Silver Spring; Charles A. Zanis; Joseph R. Crisci, both of Bowie, all of Md.

[73] Assignee: The United States of America as represented by the Secretary of the Navy

[22] Filed: Apr. 30, 1970

[21] Appl. No.: 33,454

[52] U.S. Cl..... 117/26, 73/7, 117/75,  
117/92, 117/132 CF, 117/135

[51] Int. Cl. .... B32b 15/08, B44d 1/42

[58] Field of Search..... 117/75, 132 CF, 92, 135, 26

[56] **References Cited**

UNITED STATES PATENTS

|           |         |                       |              |
|-----------|---------|-----------------------|--------------|
| 3,296,844 | 1/1967  | Quinlan .....         | 117/92 X     |
| 2,533,501 | 12/1950 | Pendleton et al. .... | 117/75 X     |
| 2,798,005 | 7/1957  | Love .....            | 117/132 CF X |
| 2,691,814 | 10/1954 | Tait.....             | 117/75 X     |

OTHER PUBLICATIONS

Fitzsimmons et al., Thin Films of PTFE Resin as Lubricants and Preservative Coatings for Metals, NRL Report, 4753, June 15, 1956, p. 16.

Primary Examiner—William D. Martin

Assistant Examiner—Ralph Husack

Attorney—Richard S. Sciascia, Louis B. Applebaum and Ernest F. Weinberger

[57] **ABSTRACT**

Minimizing the galling of titanium (or alloys) in sea water by first providing a conversion coating such as an impregnated coating of polytetrafluoroethylene, then overlaying with a coating of molybdenum disulfide and a final outer coating of asphaltic grease. An apparatus for evaluating galling of titanium wires under extreme pressure wherein a rope or wire is supported on a reciprocating weighted crank arm and abuts a stationary wire. The weighted arm applies the necessary pressure and imparts relative motion between the wires, and thereby causes repeatable galling results.

2 Claims, 4 Drawing Figures

*GALLING TESTS ON Ti 13V-11Cr-3Al  
AND VARIOUS COATINGS IN SEA WATER*

| COATING                                                                | NUMBER OF CYCLES TO FAILURE | AVERAGE NUMBER OF CYCLES TO START GALLING |
|------------------------------------------------------------------------|-----------------------------|-------------------------------------------|
| GRANO DRAW + TEFLO PASTE                                               | 3, 3, 3                     | 3                                         |
| NONE                                                                   | 1, 1                        | 1                                         |
| FLUORIDE IMPREGNATION + GREASE                                         | 2, 2                        | 2                                         |
| MOLYBDOENUM DISULFIDE                                                  | 4, 4, 1                     | 1                                         |
| TEFLON IMPREGNATION                                                    | 22, 22, 26, 25, 23, 27      | 24                                        |
| TEFLON ASPHALTIC GREASE                                                | 100, 78, 51, 85, 115, 47    | 79                                        |
| GRANO DRAW + MOLYKOTE                                                  | 26, 23, 19, 15              | 21                                        |
| GRANO DRAW + ASPHALTIC GREASE                                          | 20, 17, 15, 23, 45, 32      | 25                                        |
| TEFLON IMPREGNATION + MOLYBDOENUM SULFIDE + THIN COAT ASPHALTIC GREASE | 83, 200, 200                | 160                                       |
| IMPROVED PLOW STEEL WIRE                                               | 40, 40, 40                  | 40                                        |

Patented April 4, 1972

3,653,940

2 Sheets-Sheet 1



Fig. 1



Fig. 2



Fig. 3

INVENTORS.  
ROBERT A. OHLBAUM  
CHARLES A. ZANIS  
JOSEPH R. CRISCI  
BY  
Ernest J. Weinberger  
Don B. Gividen  
ATTORNEYS

Patented April 4, 1972

3,653,940

2 Sheets-Sheet 2

GALLING TESTS ON Ti 13V-11Cr-3Al  
AND VARIOUS COATINGS IN SEA WATER

| COATING                                                                | NUMBER OF CYCLES TO FAILURE | AVERAGE NUMBER OF CYCLES TO START GALLING |
|------------------------------------------------------------------------|-----------------------------|-------------------------------------------|
| GRANO DRAW + TEFILON PASTE                                             | 3,3,3                       | 3                                         |
| NONE                                                                   | 1,1                         | 1                                         |
| FLUORIDE IMPREGNATION + GREASE                                         | 2,2                         | 2                                         |
| MOLYBDENUM DISULFIDE                                                   | 1,1,1                       | 1                                         |
| TEFLON IMPREGNATION                                                    | 22,22,26,25,23,27           | 24                                        |
| TEFLON ASPHALTIC GREASE                                                | 100,78,51,85,115,47         | 79                                        |
| GRANO DRAW + MOLYKOTE                                                  | 26,23,19,15                 | 21                                        |
| GRANO DRAW + ASPHALTIC GREASE                                          | 20,17,15,23,45,32           | 25                                        |
| {TEFLON IMPREGNATION + MOLYBDENUM SULFIDE + THIN COAT ASPHALTIC GREASE | 83,200,200                  | 160                                       |
| IMPROVED PLOW STEEL WIRE                                               | 40,40,40                    | 40                                        |

Fig. 2

INVENTORS.  
ROBERT A. OHLBAUM  
CHARLES A. ZANIS  
JOSEPH R. CRISCI  
BY  
Ernest J. Weinberger  
John B. Cappelletti  
ATTORNEYS

## TITANIUM AND TITANIUM ALLOY WITH LUBRICANT COATED SURFACE

The invention described herein may be manufactured and used by or for the Government of the United States of America for governmental purposes without the payment of any royalties thereon or therefor.

### BACKGROUND OF THE INVENTION

#### 1. Field of the Invention

The present invention relates to coatings and means for reducing the galling under pressure between selected surfaces, and more particularly pertains to providing three overlaying coatings for titanium or alloys thereof to minimize the galling between such surfaces in sea water.

#### 2. Description of the Prior Art

In the field of coatings for metals, it has been the general practice to employ readily available coatings of various plastics and lubricants. Such materials, either alone or in combination, have been unsatisfactory in that, although they reduce titanium galling in air, they are almost entirely ineffective when the abrading wires are subjected to a salt water environment.

### SUMMARY OF THE INVENTION

The general purpose of this invention is to provide a titanium coating that has all the advantages of prior art techniques and has none of the above described disadvantages. To attain this, the present invention provides a unique combination of three individual coatings wherein the base coat is an impregnation of Teflon, the intermediate coating is molybdenum disulfide and an outer coating is of asphaltic grease, whereby galling at extreme pressures and in sea water is substantially reduced.

An object of the present invention is to provide a reliable, simple, inexpensive coating for titanium surfaces which may be readily applied and reduces galling.

Another object is to provide a special lubricating composition for titanium surfaces for the reduction of galling in sea water.

Other objects and many of the attendant advantages of this invention will be readily appreciated as the same becomes better understood by reference to the following detailed description when considered in connection with the accompanying drawings.

### BRIEF DESCRIPTION OF THE DRAWINGS

FIG. 1 is a top view of a machine employed to evaluate the galling between wires;

FIG. 2 is a side elevation of the machine of FIG. 1;

FIG. 3 is a plan view of the wires subjected to extreme rubbing pressure; and,

FIG. 4 is a list of the results of galling tests on wires coated with various compositions.

### DESCRIPTION OF THE PREFERRED EMBODIMENT

In the embodiment of the galling test machine of FIG. 1, a variable speed drive motor 10 rotatably drives an eccentric

cam 11 via shaft 12 which in turn is connected through shaft 13 to crank arm 14. This crank arm reciprocates between bearings 15 and 16 and provides simple harmonic motion. A cycle counter 17 senses the number of reciprocations of the arm and may be electrically connected to the motor 10 so as to terminate the arm movement after a preset number of cycles. The arm itself is unsupported vertically and carries at its far end a weight member 18 so as to pivot about the shaft 13 and provide an additional downward force. Disposed on the underside of the arm opposite the member 18 and attached to the arm is one of the wires 19, to be evaluated for galling.

As illustrated in FIG. 2, the motor 10 and the bearing 15 and 16 are supported by base 20, which also carries block 21 directly beneath weight 18. Disposed on the upper surface of block 21 is a stationary wire 22, which contacts wire 19 and rubs thereagainst as the arm 14 reciprocates. FIG. 3 depicts the spatial relationship of the wires or ropes under test. The moving wire 19 is shown in both of its terminal positions and the areas marked thereon indicate where the galling is taking place.

Since in one particular important application, titanium alloy wire rope is subjected to extreme galling pressure, this testing apparatus was designed to apply high pressure and may be operated in a sea water atmosphere. Additionally, wire ropes are fabricated under certain standards which set the angular relations between the strands and the ropes used in specific configurations. This determines the angular separation between the wires 19 and 22 which, in the illustrated simulation, is approximately 65°.

Galling tests of various representative coatings applied to a titanium alloy (Ti 13V-11 Cr-3Al) were performed and the results are tabulated in FIG. 4. These results clearly indicate the superior quality of applicants' coating in reducing galling in view of the average number of cycles required to start galling. Applicants first impregnate the titanium wire with polytetrafluoroethylene (PTFE - hereinafter referred to under its trade mark designation Teflon) by standard methods described by the manufacturer and supplier. This initial coating is of the conversion type and other materials such as fluorides could be used to control the porosity. This undercoating, which may also be Teflon is then covered with a layer of molybdenum disulfide which is overlayed with a common asphaltic grease.

Obviously many modifications and variations of the present invention are possible in the light of the above teachings. It is therefore to be understood that within the scope of the appended claims the invention may be practiced otherwise than as specifically described.

We claim:

50 1. A metal shape selected from the class consisting of titanium and titanium alloys having a first coating consisting essentially of polytetrafluoroethylene applied directly on the surface of the metal shape to control porosity, a second coating consisting essentially of molybdenum disulfide, and an outer 55 coating of asphaltic grease.

2. The metal shape of claim 1 wherein said first coating is an impregnation of polytetrafluoroethylene.

\* \* \* \* \*